

Nov. 24, 1925.

J. C. DAVIS

1,563,170

METHOD OF TEMPERING

Filed Oct. 24, 1923

2 Sheets-Sheet 1



Witness:

Fed Garrison

Inventor:  
James C. Davis  
by attorney  
Anne Carpenter

Nov. 24, 1925.

J. C. DAVIS

**1,563,170**

#### METHOD OF TEMPERING

Filed Oct. 24, 1923

2 Sheets-Sheet 2



Witness:

R. G. Johnson

Inventor:  
James Carey Davis  
By attorney  
John Farrenker

## UNITED STATES PATENT OFFICE.

JAMES CAREY DAVIS, OF HINSDALE, ILLINOIS.

## METHOD OF TEMPERING.

Application filed October 24, 1923. Serial No. 670,486.

*To all whom it may concern:*

Be it known that I, JAMES CAREY DAVIS, a citizen of the United States, and a resident of Hinsdale, in the county of Du Page 5 and State of Illinois, have invented certain new and useful Improvements in Methods of Tempering, of which the following is a specification.

My present invention relates to the art of 10 tempering in general, more particularly to the tempering of metal and specifically to the localized hardening of steel castings containing a modifying agent. Broadly considered, the invention comprehends an 15 improved method for tempering, an apparatus for carrying out the tempering method, and the resultant improved product.

While the invention has a broad field of usefulness for changing the state of various 20 articles of different composition, I have found it of peculiar utility for producing cast steel car wheels containing manganese as a modifying agent and I therefore find it convenient to describe the invention in connection with such a product, it being understood that such limited field of specific description is employed purely for purposes 25 of an example of the utility of the invention in its several phases.

30 The principal objects of the present invention are the provision of an improved method of tempering; the provision of an improved apparatus for tempering; the provision of an improved tempered product; the provision 35 of a method of tempering characterized by a localization of the tempering; the provision of a method of tempering wherein the area of the tempering may be substantially controlled within predetermined limits; the provision of a method of tempering characterized by the direction of fluid upon predetermined parts only of the article to be tempered; the provision of a method 40 of tempering characterized by a differential or progressive tempering of the article; the provision of a method of tempering characterized by the employment of means to prevent action of the tempering steps upon such parts of the article as it is not desired 45 to modify; the provision of a method of tempering characterized by so placing the surfaces to be tempered and so carrying out the steps of tempering that certain parts of the article upon which the operation is performed are left unchanged; the provision of 50

a method of tempering characterized by the directing of the treating fluid upon the article to be tempered, in general, and, in particular, means for directing such fluid upon the precise area desired to be acted 60 upon; the provision of a method of tempering characterized by the employment of a plurality of streams of different volume or intensity whereby areas of the article may be tempered differentially; the provision of 65 a method of tempering characterized by the provision of means whereby the article may be subjected to equivalent amounts of treating fluid at all predetermined points so that a substantial uniformity of tempering may 70 be attained; the provision of an improved apparatus for carrying out the several objects set forth; the provision of a tempering apparatus characterized by means for a localization of the tempering, in general, 75 and more particularly means whereby the area of tempering may be substantially limited; the provision of tempering apparatus characterized by the provision of means for ejecting the tempering fluid upon a predetermined point or points in general, and, in particular, by the employment of a plurality of ejector members so arranged that the article may be tempered differentially or 80 progressively and thus predetermined varying qualities imparted thereto; the provision in a tempering apparatus of means for preventing tempering action upon the parts of the article which it is not desired to change; the provision of a tempering apparatus 85 characterized by the horizontal ejection of the tempering fluid so that parts of the object may remain unmodified; the provision of a tempering apparatus characterized by the employment of a plurality of series 90 of streams of tempering fluid, in general; and in particular, one wherein the volumes of fluid of the several streams differ and thus the action thereof may be varied differentially or progressively; the provision of a tempering apparatus characterized by the employment of a shield protecting the article acted upon from the action of the tempering fluid, and the provision of improved means for operating such shield, together with such further objects, benefits and advantages as may hereinafter appear or may be pointed out. The word "tempering" as employed herein relates to changing the state of the metal treated, that is, may 100 105 110

apply to either hardening or softening or changing the relative state or condition of various portions of a single casting, as will appear, the example illustrated and described being for the purpose of producing a casting having various degrees of hardening in a particular region thereof.

In the attainments of the foregoing objects and certain additional benefits and advantages to be hereinafter disclosed, I find it convenient to carry out my improved method by means of an apparatus, one embodiment of which is illustrated in the accompanying drawings.

On inspection of these drawings it will be observed that as above suggested, I have for purposes of convenience in disclosure and description illustrated an apparatus of a form adapted for the treatment of a disc-like metallic casting, to-wit: in the present case, a flanged cast manganese-steel wheel. The invention is peculiarly adapted for the treatment of such objects, as will be manifest when it is considered that a great desideratum in the hardening of wheel treads is that such hardening be both uniform in order that the wheel may wear uniformly in service, and not become out-of-round, and at the same time that the hardening be localized to that portion of the tread and throat which is most usually in contact with the rail head, in order that the rim of the wheel may wear uniformly and not become grooved in service. To this end therefore it is most desirable that the flange of the wheel which ordinarily is of quite sufficient hardness without tempering be not further hardened, and similarly that the outer marginal portion of the tread which is opposite to the flange and receives much less wear, owing to its relatively less contact with the rail head, be left unmodified and relatively soft so that the wheel tread in service will wear down uniformly. It is likewise desirable that the web and center of the wheel be left free from hardening and in their relatively soft state.

In the accompanying drawings—

Figure 1 is a plan view of the tempering apparatus;

Figure 2 is a sectional view taken on the line II—II of Figure 1, the wheel being shown therein in elevation;

Figure 3 is a fragmentary sectional plan view of a part of the apparatus in Figure 1; and

Figure 4 is a transverse sectional view of the wheel tread.

Referring first more particularly to Figures 1 and 2 of the drawings it will be observed that the tempering apparatus here shown comprises an elliptically formed casing 10 provided with a chamber 11 having connections to sources of fluid 12, baffle plates 10<sup>a</sup> being disposed in said casing 10 adjacent

the inlets 13 of the fluid connections 12, in order to prevent surging of the fluid through the adjacent jets shortly to be described. The baffle plates 10<sup>a</sup> are provided with suitable ports 14 for the equalization of fluid pressure within said casing 10, to the end that the discharge through the several jets may be substantially uniform, and clean-out openings above inlets 13 are provided, with closing plugs 13<sup>a</sup>.

In order that, where desired, as in the case of a wheel tread, the article acted upon may be tempered uniformly, I find it convenient to impart to the chamber 15 within the casing 10 a contour corresponding in general to that of such article, thus in the present case, since a wheel tread is to be acted upon, the chamber 15 is annular.

For directing fluid from the chamber 11 of the casing 10 to the surface to be treated, in the present instance the tread 16 of the wheel 17, I employ a number of streams or jets of fluid which are conveniently given the desired direction by means of nozzles 18. The latter, as will be apparent on viewing Figure 1, are preferably arranged radially and directed towards the center of the wheel, which is to be carefully centered in the casing 10 and may be sustained by the supporting members 19. As will be seen on viewing Figure 2, the nozzles 18 are preferably arranged in a plurality of series, 20, 21, 22. In the present case inasmuch as the object is to harden the throat 23 and tread 16 of the wheel, I find it desirable to eject the largest quantity of fluid through the nozzle series 20, a lesser quantity through the nozzle series 21 and the least quantity through the nozzle series 22. To this end the series 20 contains the largest number of nozzles and the series 21 and 22 progressively less numbers thereof.

At various times and for various purposes, and especially in the present case of a wheel tread it is desirable to preserve a certain part of the article acted upon from the tempering action of the fluid streams emitted from the jet series 20, 21, 22. For the accomplishment of this purpose I have provided the shield 24, which when used for protecting an article which is circular in cross section may be a band of springy metal such as is indicated at 24 (Figure 3). One end of this band 25 may be attached to a crank arm 26, the opposite end of the band 27, passing through a stirrup 28 on such arm 26, may be attached to the casing 10 at a convenient point such as indicated at 29.

For the purpose of contracting the band 24 upon the article to be treated, e. g. the wheel 17, an operating lever 30 connected by the link 31 to the arm 26, may be employed. To facilitate one action of the shield, e. g. its contraction, a tension spring 32 having a suitable connection to the exterior of the cas-

ing at a convenient point such as is indicated at 33, may be utilized.

From the foregoing description of my improved method of and apparatus for tempering, it will be perceived that the resultant product may be tempered as desired, that such tempering may be localized, that such tempering may be uniform, as for example, in belts around a cylindrical object such as a wheel tread, and that by its use belts of differing hardness may be produced, such as those indicated by the index numbers, according to the Brinell hardness scale appearing on the inner periphery, the flange, the throat, the tread 16 and the outer periphery 34 of the wheel whose contour in cross-section is outlined in Figure 4, and all this without affecting such parts as may be desirably left unchanged.

20 Other advantages and uses of my present invention will occur to those who are skilled in the art.

Having thus described my invention and illustrated its use, what I claim as new and 25 desire to secure by Letters Patent is:

1. The method of tempering a continuous surface of metal which includes directing against the metal a plurality of series of streams of fluid to strike the metal independently.

2. The method of tempering a continuous surface of metal which includes directing against the metal at spaced points a plurality of series of streams of fluid to strike 35 the metal independently.

3. The method of tempering metal which includes directing a plurality of series of streams of fluid against the metal, the several series varying in volume.

40 4. The method of tempering metal which includes directing a plurality of series of streams of fluid against the metal, an upper series having more volume than a series therebelow.

45 5. The method of tempering a continuous surface of metal which includes directing a plurality of series of streams of fluid against the surface of said metal, the number of streams in two of the series varying to strike 50 the metal independently.

55 6. The method of tempering metal which includes directing a plurality of series of streams of fluid against the metal, the volume of streams in the several series varying progressively.

7. The method of tempering a continuous surface of metal which includes directing a plurality of streams simultaneously upon different portions of the surface of said 60 metal to strike the metal independently.

8. The method of tempering a continuous surface of metal which includes directing a plurality of streams upon different portions of the surface of said metal, said streams 65 having similar relation to the periphery of

the casting to strike the metal independently.

9. The method of tempering a continuous surface of metal which includes directing a plurality of streams upon different portions 70 of the surface of said metal, said streams having similar relation to the center of the casting to strike the metal independently.

10. The method of tempering a continuous surface of metal which includes directing a 75 plurality of streams radially upon different portions of the surface of said metal to strike the metal independently.

11. The method of hardening the tread portion of a wheel which includes the step 80 of subjecting a wheel tread, part of which is shielded from a tempering fluid, to a stream of fluid directed upon such tread.

12. The method of hardening the tread portion of a flanged wheel which includes 85 the step of subjecting a wheel tread, part of which is shielded from a tempering fluid, to a stream of fluid directed upon such tread at a point adjacent the flange thereof.

13. The method of hardening the tread 90 portion of a wheel which includes the step of subjecting a wheel tread, part of which is shielded from a tempering fluid, to a plurality of symmetrically arranged streams of fluid.

14. The method of hardening the tread portion of a wheel which includes the step 95 of subjecting the tread of a wheel lying on its side, and part of which tread is shielded from a tempering fluid, to a plurality 100 of streams of fluid.

15. The method of hardening the tread portion of a wheel which includes the step 105 of subjecting the tread of a wheel lying on its side, and part of which tread is shielded from a tempering fluid, to a plurality of series of streams of fluid arranged one above the other, the topmost series having the largest volume of streams.

16. As a new article of manufacture, a 110 cast steel wheel having a flange and a tread portion additionally and differentially hardened.

17. As a new article of manufacture, a heat treated cast manganese steel wheel 115 having a flange and provided with a tread and throat portions additionally hardened.

18. As a new article of manufacture, a heat treated flanged cast manganese steel wheel having tread and throat portions hardened after casting, the web of the wheel 120 being unaltered by the hardening operation.

19. As a new article of manufacture, a heat treated flanged cast manganese steel 125 wheel having its tread portion hardened after casting by localized quenching, that portion of the wheel opposite to the flange being protected from the quenching operation and remaining substantially unaltered. 130

20. As a new article of manufacture, a casting having a peripheral tempered belt, whose width is of varying hardness.

21. As a new article of manufacture, a car wheel having its cylindrical portion tempered in belts of varying degrees of hardness.

22. As a new article of manufacture, a substantially cylindrical casting having a part of its cylindrical portion tempered in varying degrees and a part of such cylindrical portion untempered.

23. As a new article of manufacture, a

cast steel wheel, having a tread and a flange thereof of predetermined degree of hardness, and a tread of said wheel being hardened to substantially the same degree as said flange.

24. As a new article of manufacture, a steel wheel having an integral tempered tread portion, another portion of the tread being untempered.

In testimony whereof I have hereunto signed my name.

JAMES CAREY DAVIS.